

## UNITED STATES PATENT OFFICE

2,654,702

ELECTRODEPOSITION OF METAL FROM  
ALKALINE CYANIDE BATHHerbert K. De Long, Midland, Mich., assignor to  
The Dow Chemical Company, Midland, Mich.,  
a corporation of DelawareNo Drawing. Application September 3, 1948,  
Serial No. 47,745

8 Claims. (Cl. 204—46)

1

The invention relates to improvements in the art of electroplating metal, particularly the electrodeposition of copper, silver and gold in aqueous alkaline cyanide plating baths.

I have discovered that inorganic fluorides, especially the alkali metal and ammonium fluorides, exert a marked beneficial effect on the electrodeposited plates of copper, silver and gold when present in substantial amount in the conventional aqueous alkaline cyanide plating baths of these metals. One of the principal advantages which results from the use of the inorganic fluoride in accordance with the invention is in increasing the brightness of the deposit. Another advantage is the reduction of pitting or immersion corrosion. These advantages obtain more especially in the plating of magnesium and its alloys, particularly when first coated with zinc by the immersion coating process described in my copending application Serial No. 778,283, filed October 6, 1947, now U. S. Patent 2,526,544.

The fluorides I prefer to use are either potassium fluoride (KF) or ammonium bifluoride (NH<sub>4</sub>F·HF), and amounts in the order of about 5 to 100 grams per liter of plating solution may be used. Preferred concentrations are in the range of about 20 to 60 grams per liter. In the following tabulations examples of plating baths compounded in accordance with the invention are set forth, together with appropriate operating conditions.

## Example I

## Copper plating bath:

|                         |                 |
|-------------------------|-----------------|
| Copper cyanide          | 41.3 g. p. l.   |
| Potassium cyanide       | 70.             |
| Rochelle salt           | 60.             |
| Potassium fluoride      | 60.             |
| Temperature             | 120° C.         |
| pH                      | 10.8.           |
| Cathode current density | 15 amp./sq. ft. |

## Example II

## Copper plating bath:

|                         |                 |
|-------------------------|-----------------|
| Copper cyanide          | 120 g. p. l.    |
| Sodium cyanide          | 135.            |
| Potassium hydroxide     | 42.             |
| Sodium thiocyanate      | 15.             |
| Betaine                 | 1.5.            |
| Potassium fluoride      | 60.             |
| Temperature             | 160 to 180° F.  |
| pH                      | 12.5 to 13.5.   |
| Cathode current density | 15 amp./sq. ft. |

2

## Example III

## Copper plating bath:

|                         |                 |
|-------------------------|-----------------|
| Copper cyanide          | 26.25 g. p. l.  |
| Sodium cyanide          | 32.5.           |
| Sodium carbonate        | 30.             |
| Ammonium bifluoride     | 1 to 10.        |
| Temperature             | 120° C.         |
| pH                      | 9.5 to 11.0.    |
| Cathode current density | 20 amp./sq. ft. |

## Example IV

## Silver plating bath:

|                         |                 |
|-------------------------|-----------------|
| Silver cyanide          | 30 g. p. l.     |
| Potassium cyanide       | 41.2.           |
| Potassium carbonate     | 45.             |
| Potassium fluoride      | 30.             |
| Temperature             | 70-80° F.       |
| pH                      | 10.5 to 12.0.   |
| Cathode current density | 20 amp./sq. ft. |

## Example V

## Silver plating bath:

|                         |                 |
|-------------------------|-----------------|
| Silver cyanide          | 24 g. p. l.     |
| Sodium cyanide          | 19.             |
| Potassium nitrate       | 112.5.          |
| Potassium fluoride      | 30.             |
| Temperature             | 70 to 80° F.    |
| pH                      | 10.5 to 12.0.   |
| Cathode current density | 20 amp./sq. ft. |

## Example VI

## Gold plating bath:

|                         |                   |
|-------------------------|-------------------|
| Potassium gold cyanide  | 3.75 g. p. l.     |
| Potassium carbonate     | 7.5.              |
| Potassium cyanide       | 3.75.             |
| Potassium fluoride      | 30.               |
| Temperature             | 70-80° F.         |
| pH                      | 10.5-12.0.        |
| Cathode current density | 5-15 amp./sq. ft. |

In the foregoing examples the plating bath compositions, except for the fluoride constituent, are conventional. It will be understood that these examples are illustrative and are not to be taken as limitative of the invention. The essential requirements of the plating baths are the presence as the cyanide in water solution of the metal to be deposited, together with sufficient alkalinity to maintain the pH in the range of about 9 to 13, and, in accordance with the invention, the fluoride constituent is included. Insofar as the pH is concerned it is preferable to operate the copper plating baths at a pH be-

tween about 10 and 13 and the silver and gold baths at a pH between about 9 and 12. This alkalinity is readily obtained by the addition to the plating bath of an alkali metal hydroxide or carbonate such as NaOH, KOH, K<sub>2</sub>CO<sub>3</sub> and Na<sub>2</sub>CO<sub>3</sub> or ammonium hydroxide. The presence of free cyanide (CN) in addition to that furnished by the cyanide of the metal to be deposited is desirable. This may be supplied by including in the bath an alkali metal cyanide such as sodium cyanide and potassium cyanide in amount such as to yield from about 2 to 5 grams of CN per liter.

In plating magnesium and its alloys in aqueous alkaline cyanide baths containing fluoride in accordance with the invention, it is advantageous first to deposit a film of zinc upon the work as described in my patent application aforementioned. This may be accomplished, for example, by immersing for 5 minutes the article to be plated in the following bath maintained at about 180° F.:

Zinc immersion coating bath:

|                                               |       |      |            |
|-----------------------------------------------|-------|------|------------|
| Na <sub>4</sub> P <sub>2</sub> O <sub>7</sub> | grams | 10.0 | 25         |
| ZnSO <sub>4</sub> ·7H <sub>2</sub> O          | do    | 4.0  |            |
| KF                                            | do    | 1.0  |            |
| K <sub>2</sub> CO <sub>3</sub>                | do    | 0.5  |            |
| Water sufficient to make 100 grams of         |       |      |            |
| solution                                      |       |      |            |
| pH of solution                                |       |      | About 10.2 |

The immersion results in an adherent zinc deposit upon which copper, silver, or gold may be electroplated from the aqueous alkaline cyanide plating baths described above. In using the zinc immersion coating the coated article need only be rinsed with water before proceeding with the electroplating operation.

In some instances, in forming deposits of copper, silver and gold on magnesium and its alloys it is desirable to apply a strike of either copper or silver over the zinc coating before proceeding with the plating operation. As a copper strike the following bath may be used:

|                                              |          |
|----------------------------------------------|----------|
| Copper strike bath:                          | G. p. 1. |
| Copper cyanide                               | 41.3     |
| Sodium cyanide                               | 50.8     |
| Sodium carbonate                             | 30       |
| Rochelle salts                               | 45       |
| Sodium thiosulphate                          | 1.9      |
| (pH about 10 to 11.)                         | 50       |
| Cathode current density 5 to 10 amp./sq. ft. |          |
| for 2 to 3 minutes followed by an increase   |          |
| of current density to 15 amp./sq. ft. for    |          |
| about 3 minutes.                             |          |

The presence of the soluble fluoride in the alkaline cyanide plating bath has the advantage of reducing or preventing immersion deposition and attack upon the work. Attack is sometimes revealed by the presence of a smutty film on the work and the formation of pits. The electro-

plates obtained in the presence of the fluoride are brighter, and pitting of the work due to corrosion by the bath is overcome.

I claim:

1. In a method of depositing an electroplate of a metal selected from the group consisting of copper, silver, and gold upon articles of magnesium and magnesium alloys from an aqueous alkaline cyanide plating solution having a pH of 9 to 13 and containing a cyanide of one of the metals selected from the group consisting of copper, silver, and gold and from 2 to 5 grams per liter of CN provided by an alkali metal cyanide by electrolyzing the solution with the article as cathode whereby the selected metal is electro-deposited on the article, the improvement which consists in dissolving in the plating solution a water-soluble inorganic fluoride selected from the group consisting of the alkali metal and ammonium fluorides in amount from 5 to 100 grams per liter of the plating solution.

2. The method according to claim 1 in which the water-soluble inorganic fluoride is ammonium fluoride.

3. The method according to claim 1 in which the water-soluble inorganic fluoride is an alkali metal fluoride and the metal to be deposited as an electroplate is copper.

4. The method according to claim 1 in which the water-soluble inorganic fluoride is an alkali metal fluoride and the metal to be deposited as an electroplate is silver.

5. The method according to claim 1 in which the water-soluble inorganic fluoride is an alkali metal fluoride and the metal to be deposited as an electroplate is gold.

6. The method according to claim 1 in which the water-soluble inorganic fluoride is ammonium fluoride and the metal to be deposited as an electroplate is copper.

7. The method according to claim 1 in which the water-soluble inorganic fluoride is ammonium fluoride and the metal to be deposited as an electroplate is silver.

8. The method according to claim 1 in which the water-soluble inorganic fluoride is ammonium fluoride and the metal to be deposited as an electroplate is gold.

HERBERT K. DE LONG.

References Cited in the file of this patent

UNITED STATES PATENTS

| Number    | Name    | Date           |
|-----------|---------|----------------|
| 946,903   | Kern    | Jan. 18, 1910  |
| 2,449,726 | Slatkin | Sept. 21, 1948 |

OTHER REFERENCES

- Bandes, Trans. of Electrochemical Society, vol. 88 (1945), pp. 265-9.  
 Sanigar, Trans. of Electrochemical Society, vol. 59 (1931), pp. 307-8, 324-7.